

Feb. 5, 1946.

H. B. KLINE ET AL

2,394,519

MANUFACTURE OF THREAD OR THE LIKE

Filed July 29, 1940

3 Sheets-Sheet 1



Feb. 5, 1946.

H. B. KLINE ET AL  
MANUFACTURE OF THREAD OR THE LIKE

2,394,519

Filed July 29, 1940

3 Sheets-Sheet 2

FIG. 2



Feb. 5, 1946.

H. B. KLINE ET AL

2,394,519

MANUFACTURE OF THREAD OR THE LIKE

Filed July 29, 1940

3 Sheets-Sheet 3



## UNITED STATES PATENT OFFICE

2,394,519

## MANUFACTURE OF THREAD OR THE LIKE

Hayden B. Kline and Louis S. Fryer, Cleveland,  
and Robert D. MacLaurin, Bay Village, Ohio,  
assignors to Industrial Rayon Corporation,  
Cleveland, Ohio, a corporation of Delaware

Application July 29, 1940, Serial No. 348,232

7 Claims. (Cl. 18—54)

This invention relates to the manufacture, by the extrusion of a coagulable mass into a liquid which serves to solidify it, of strands, strips, sheets, tubes, threads, filaments, etc., hereinafter referred to as "thread." More particularly, the invention relates to the treatment of such liquid for the purpose of rendering substantially innocuous otherwise objectionable substances formed by the coagulable mass and coagulating liquid during coagulation operations. For convenience, the invention will be described in connection with the manufacture of multiple filament viscose artificial silk thread, although it may be employed to advantage, at least in certain of its aspects, in connection with the manufacture of other products formed by the extrusion of a coagulable mass into a coagulating liquid.

Multiple filament artificial silk viscose thread is formed by extruding an aqueous solution of sodium cellulose xanthate ("viscose") through a multiple-orifice spinneret of noble metal or noble metal alloy into an acidic coagulating liquid. The coagulating liquid ordinarily includes sulfuric acid, sodium sulfate, a small amount of zinc sulfate, and, if desired, other beneficial substances. After its extrusion from the spinneret, the sodium cellulose xanthate reacts to form, on one hand, the regenerated cellulose of which the thread is primarily composed and, on the other, such by-products as sodium sulfate, carbon disulfide, hydrogen sulfide and free sulfur, some of which are undesirable. Sundry impurities; viz., hemi-cellulose, complex sulfur compounds, and insoluble compounds of silicon, lead, zinc and occasionally nickel are also introduced into the thread-forming system from the viscose and other sources.

If such substances are not rendered substantially innocuous by continuous removal of the impurities from the coagulating liquid, their presence will soon cause serious operating difficulties. The concentration of such impurities, and hence the magnitude of the resulting difficulties, tends to increase rapidly during the coagulation operation as a result of the necessity, at least in commercial practice, of repeatedly recirculating and reusing the coagulating liquid. Because of the large amount of relatively expensive coagulating liquid employed per unit of thread, it is commercially impracticable to use the coagulating liquid only once and then discard it. The nature of the difficulties brought about by this state of affairs is well understood in the art but will be described briefly hereinafter.

Insoluble impurities, such as sulfur, cause trouble when the viscose of which the thread is to be formed is extruded through the spinneret. Unless special precautions are taken, the orifices in the spinneret soon become clogged or fouled by insoluble substances which deposit in crater-like formations around the orifices on the face of the spinneret. At the same time, ring-like deposits tend to form within the spinneret orifices: such ring-like formations appear to be caused primarily by substances in the viscose, such as cellulose, hemi-celluloses, silicates, etc., which precipitate in the spinneret orifices on being subjected to the action of the acid coagulating liquid. Deposits so formed in and about the spinneret orifices tend to reduce the denier of the individual filaments and often to block the orifices completely. In the course of the spinning operation, these factors cause considerable difficulty, usually producing broken filaments or snarls of the type known to the trade as "fishhooks."

It is not unusual under ordinary spinning conditions to have to replace 20 per cent or more of the spinnerets for such reasons each twenty-four hours. Inasmuch as a plant of moderate size will have about 10,000 spinnerets in operation at one time, this means that a very substantial amount of time and labor is lost in making replacements. The economic loss is great even in discontinuous processes of manufacturing viscose artificial silk thread; i. e., in pot- and spool-spinning processes in which the thread passes directly from the spinneret to a collecting device of limited capacity. The difficulties arising out of such conditions and the economic waste accruing therefrom are, however, vastly greater when viscose artificial silk thread is produced by so-called continuous processes.

In the continuous process, the thread proceeding from the spinneret to the collecting device is subjected to processing treatment on a series of thread-advancing devices each of which continuously but temporarily stores the thread in a large number of generally helical turns. When, in such a process, a thread breaks because of a clogged or fouled spinneret or is intentionally broken for necessary cleaning or replacement of the spinneret, all of the thread store devices to which the thread would subsequently pass, which may be as many as ten or more, must again be threaded up; that is to say, the leading end of the thread must be passed in sequence to each of said devices and caused to wind thereon in the required number of generally helical turns.

Thread leaving the coagulating bath usually tends to carry with it extraneous substances present in the coagulant. If such substances are of sufficient concentration, they may interfere with the after-treatment of the thread, as, for example, by causing objectionable side reactions. Under other conditions, they deposit on parts of the apparatus with which the thread comes into contact, forming incrustations which damage the thread. In continuous processing apparatus, interference with the after-treatment of the thread and the formation of such deposits are most likely to occur on the thread-advancing devices. The thread passes to such devices from the coagulating liquid within a very short time after its formation and is stored thereon during after-treatment for a sufficient period of time to favor the formation of such deposits or incrustations.

It is apparent, therefore, that the presence in the coagulating bath of impurities and by-products of the coagulation reaction is responsible for many operating difficulties.

The usual method of treating the coagulating liquid for the purpose of removing detrimental substances is to filter it. This, however, requires considerable liquid storage space, highly efficient filtration facilities, and the expenditure of a not inconsiderable amount of time and labor to maintain the equipment in operating condition. Moreover, even after the coagulating liquid is filtered, clogging or fouling of spinnerets tends to occur because of the presence of insoluble substances formed by the reactions which take place in the course of the solidification of the thread. Because of the colloidal character of certain of the substances present in the coagulating bath, particularly sulfur, it is sometimes difficult, if not actually impossible, to remove such substances by filtering operations.

All such difficulties, arising from the presence of impurities in the coagulating liquid or viscose, are obviated by the present invention, according to one aspect of which a water-insoluble substance, preferably an oleaginous substance, is incorporated in finely dispersed condition in the coagulating liquid. One or more suitable dispersing or emulsifying agents, which likewise may be, but are not necessarily, of the nature of an oleaginous material, are preferably employed to aid in forming a stable dispersion of the first-mentioned oleaginous material. Indeed, the dispersion of oleaginous material in the coagulating liquid may be so complete as to constitute an emulsoid. The presence in the coagulating liquid of such material or materials operates as herein-after explained to render innocuous the relatively high content of impurities present in the thread forming system, particularly in the coagulating liquid: among other things, such material or materials tend to inhibit the formation of harmful deposits not only in and upon the spinnerets but also upon other parts of the apparatus.

Under suitable circumstances, such material or materials will form a sludge, floating, suspended, or precipitated, in which sludge is contained a substantial proportion of the detrimental substances present in the coagulating liquid. Such sludge may be removed from the coagulating liquid either continuously or from time to time. Among other impurities, considerable amounts of sulfur may be separated in this manner from the coagulating liquid. Thus the necessity of filtering the coagulating liquid may be entirely eliminated; indeed, the same coagulating liquid

may be reused indefinitely without fouling spinnerets, guides, thread-advancing devices, etc.

For purposes of illustration, the invention will be described in connection with the manufacture of multiple filament viscose artificial silk thread on apparatus of the type disclosed in application Serial No. 7,114 (Patent 2,225,642), filed February 18, 1935, by W. F. Knebusch and A. H. Burkholder.

In the accompany drawings, Figure 1 represents a sectional elevation from line 1—1 of Figure 2 of a portion of such apparatus including the thread-forming portion together with certain of the after-treatment stages. Figure 2 is a front elevation of said portion of the apparatus from line 2—2 of Figure 1, some of the parts intermediate the ends of the apparatus being omitted for convenience of illustration. Figure 3 is a diagram of a preparation and circulation system for handling the coagulating liquid according to the present invention. Figure 4 is an isometric representation of a settling tank which may be employed in connection with the system shown in Figure 3. Figure 5 is a representation of a modified portion of said tank.

In the apparatus illustrated in Figures 1 and 2, threads 1 are formed by the extrusion of viscose through spinnerets 2 disposed in coagulating bath 3 contained in trough 4. Thread 1 from each spinneret passes in turn to each of a plurality of thread-advancing devices 5, 6, 7, 8, 9, etc., which, in the preferred embodiment of the invention, take the form of cantilever thread-advancing reels similar to that shown in said Patent 2,225,642. The reels are preferably disposed in stepped arrangement with the unsupported ends of all reels on the same side of the apparatus extending toward the corresponding operating face of the machine, so that the thread-discharge end of each reel may be in apposition to the thread-receiving end of the succeeding reel.

Interposed between successive thread-advancing reels, and also between spinneret 2 and reel 5, are thread guides 10. Such guides, which may take any suitable form, serve in each case to guide the thread to the thread-receiving end of the reel to which it is desired that the thread shall pass. Between reel 5 above coagulating trough 4 and reel 6 below said trough, thread 1 travels through a vertical channel 11 mounted in juxtaposition to the coagulating trough. Channel 11 provides an open, unobstructed passageway for the thread in its travel from reel 5 to reel 6.

In the apparatus illustrated in the drawings, a plurality of thread-producing units, each of which comprises a spinneret 2, a reel 5, a channel 11, a series of reels 6, 7, 8, 9, etc., and associated apparatus, is disposed along each side of a common longitudinally extending coagulating trough 4. By an arrangement of this type, a large thread-production capacity can be obtained in a very compact space. As is apparent from Figures 1 and 2, corresponding parts of the thread-producing units on each side of the apparatus are disposed in corresponding positions lengthwise of the apparatus, thereby providing operating and constructional advantages.

In the illustrated apparatus, no processing medium of any kind is applied to the thread on the reel above the coagulating trough: said reel serves simply to store the thread for a period long enough to permit coagulation of the freshly spun thread to proceed substantially to comple-

tion. However, additional coagulating liquid may be, and preferably is, applied to thread 1 while it is on reel 6. Washing liquid may be applied to the thread on reel 7; desulfurizing liquid on reel 8; washing liquid on reel 9, etc. In this manner, all of the desired processing treatments may be performed upon the thread.

It will be noted that in each case the liquid is applied to the thread on the reel from a reagent distributing tube 12 which communicates with a supply conduit 13 extending longitudinally of the apparatus above the horizontal series of reels of which such reel forms a part: said conduit may be supplied with processing liquid from any suitable source. Below each of the reels on which processing liquid is applied to the thread is disposed a collecting trough 14 which likewise extends lengthwise of the apparatus. Each of said collecting troughs may communicate with the sewer or, if desired, with make-up and recirculating means for the processing liquid.

In the apparatus of Figures 1 and 2, reels 6 to 9, inclusive, of each downwardly-extending series of reels are positively rotated, as by means of inclined drive shaft 15 and gears 16, from a drive shaft 17 extending longitudinally of the apparatus along each side thereof. On both sides of the apparatus, the reels 5 disposed above the coagulating trough are driven by means of gears contained in gear boxes 19 from a common longitudinally-extending drive shaft 18. Drive shafts 17 and 18 are driven from common drive means in housing 21 which drive means also rotates drive shafts 22, one of which is disposed along each side of the apparatus for the purpose of driving viscose pumps 23. Viscose pumps 23 are supplied with viscose from a longitudinally-extending conduit 24, each pump serving to convey the viscose to its associated spinneret 2 through tube 25 and mass tube 26.

While the coagulating liquid 3 contained in trough 4 may be supplied and recirculated by various means, that shown in the illustrated embodiment of the invention has been found to be particularly satisfactory.

As is apparent from Figures 1, 2 and 3, the coagulating liquid is supplied to the coagulating trough 4 from means disposed at one end thereof. The liquid is pumped to an elevated supply box 27 at said end, from each side of which box 27 it flows through a weir notch 28 into a corresponding compartment 29. A substantially constant pressure of liquid is thus maintained in supply conduits 32, one of which extends longitudinally of the coagulating trough 4 along one side thereof and communicates with one of the compartments 29. Openings 33 are provided along said conduits 32 to permit the coagulating liquid to flow into the trough at spaced points.

The liquid flows out of coagulating trough 4 through drain conduits 34 disposed in such trough at intervals therealong. Such drain conduits communicate with a common discharge conduit 35. Preferably the inlet to each of said drain conduits 34 is disposed, as shown, at a sufficient distance above the bottom of the trough to maintain the liquid level in the trough at the desired height. Suitable trap or strainer means 36 are provided at the inlet to prevent entrance into the discharge ducts of material which might clog them.

As shown diagrammatically in Figure 3, supply box 27 is provided with an overflow conduit 37 which serves as an emergency drain should the liquid be supplied to said box at a rate greater

than that at which it is removed therefrom. Coagulating liquid leaving trough 4 through conduits 34 and 35 passes to what might be termed a make-up tank 38 from which it flows through conduit 39 to a storage tank 41, a valve 42 being provided in said conduit 39 to regulate the flow. From storage tank 41 the liquid is pumped by pump 43 to supply box 27 through conduit 44, thus completing the recirculating cycle. If desired, a valve 45 may be provided between the tank 41 and pump 43 to regulate the flow of fluid from the tank to the supply box.

Because of the addition to the system of extraneous liquids, such as water present in the viscose which is being coagulated, a conduit 46 is provided which, through regulating valve 47, may be used to bleed off any desired amount of liquid from discharge conduit 35.

Sodium sulfate, one of the by-products of the coagulation reaction, tends to increase in amount because of the fact that it is being continuously formed as a result of the reaction. The addition of water present in the viscose being coagulated dilutes the solution; consequently, if no other precautions were to be taken, the sodium sulfate would eventually reach and maintain an equilibrium concentration of about 15%. It is usually desired to have a higher concentration of sodium sulfate; e. g., about 20%, by weight, in the coagulating liquid. Accordingly, as in the case of most commercially used coagulating baths, it is necessary to increase the concentration of sodium sulfate by suitable means.

In the illustrated embodiment of the invention, this is done without the addition of sodium sulfate from any external source by continuously bleeding off through conduit 48 a portion of the coagulating liquid which passes through conduit 44 on its way to coagulating trough 4. The portion so bled off is conducted to an evaporator 49, indicated diagrammatically in Figure 3. The evaporator, by removing some of the water, increases the concentration of sodium sulfate and other involatile substances in the coagulating liquid. The concentrated liquid is then passed through conduit 51 to make-up tank 38. Valves 52 are provided to regulate the flow of liquid through evaporator 49 which is operated under such conditions that the concentration of sodium sulfate in the liquid passing through conduit 51 is maintained at the desired value.

From time to time, or, if preferred, continuously, reagents may be supplied to replace those consumed in the coagulation reaction or removed with the portion of liquid bled off through conduit 46. In the circulation system of Figure 3, such additions are made in make-up tank 38. Concentrated sulfuric acid, for example, may be supplied from a container 53 through a line 54 embodying a regulating valve 55. Water may, if needed, be added from a tank 56 through a suitable conduit 57. Zinc sulfate may be added in solid form or in aqueous solution. In the system illustrated, such solution is supplied to make-up tank 38 from a tank 58 through conduit 59 embodying regulating valve 60. Means may also be provided for adding sodium sulfate. For use in the illustrated apparatus, the coagulating liquid may include, in addition to the above indicated amount of sodium sulfate, 10% to 11% of sulfuric acid and .3% to .5% of zinc as zinc sulfate.

Preferably, heating means, such as steam coils 61, are provided in storage tank 41 to heat the coagulating liquid so that when in the coagulating trough 4 it is at about 45° C.

As shown in Figure 4, storage tank 41 is divided by a partition 64 into a large compartment 62 and a small compartment 63. The coagulating liquid is admitted to the large compartment of the tank by means of conduit 39 and leaves the tank through a conduit 44 communicating with the small compartment. Partition 64 is provided with a weir notch 65 through which the liquid from the large compartment overflows into the small compartment. In the embodiment of the invention shown in Figure 4, a removable baffle plate 66, preferably of semi-circular cross section, is disposed above said weir notch 65 to prevent floating sludge from overflowing from the liquid in large compartment 62 into small compartment 63.

The system shown diagrammatically in Figure 3 contemplates the thorough mixing together of the coagulating liquid and the oleaginous material to which reference has already been made, to which end a previously prepared aqueous dispersion of the latter is introduced into the former in the small compartment 63 of storage tank 41 by means of pipe 67. The high degree of turbulence in small compartment 63 caused by the overflowing of the liquid at weir notch 65 of partition 64 serves to mix the oleaginous material with the coagulating liquid. The previously prepared dispersion of the oleaginous material is made up in the first instance in mixing tank 68, which may be any one of several known types of mixing tanks provided with an electrically or mechanically operated agitator. To such mixing tank, the oleaginous material or materials, and, if desired, a dispersing agent, may be supplied from suitable sources, such as tanks 69, 70 and 71. Thus, in one instance, a highly refined petroleum oil ("white oil") may be supplied from tank 69 through conduit 73, while from tank 70 a less highly refined petroleum oil ("mineral oil") may be supplied through conduit 74. Of course, an appropriate quantity of a single oil of suitable characteristics may be added instead. Preferably, an emulsifying agent which will cause such oleaginous liquid or liquids to form a stable aqueous emulsion is added from container 71 through conduit 75. Water is added through line 72 in such quantities as may be needed.

The substance sold by the Standard Oil Co. of Ohio under the trade-name "Sohio-X Soluble Oil," which substance is understood to be an alkali metal salt of a sulfonated hydrocarbon oil, has been found to be a satisfactory emulsifying agent. This substance, which is soluble in water, is substantially insoluble in the coagulating liquid, but nevertheless gives a finely dispersed emulsion of mineral oil. Preferably, the emulsion is made up in the following manner: approximately 600 pounds of white oil (80 seconds Saybolt viscosity at 100° F.), 600 pounds of No. 17 mineral oil (80 seconds Saybolt viscosity at 100° F.), and approximately 30 pounds of an approximately 20% aqueous solution of Sohio-X Soluble Oil are mixed with enough water to bring the total weight of the mixture up to 2000 pounds.

The prepared emulsion to be added to the coagulating liquid thus contains, by weight, about 60% of petroleum oil emulsified by approximately .3% of an emulsifying agent in about 39.7% water. In other words, in the present example, the petroleum oil is emulsified by an emulsifying agent added in the proportion of about .5%, based on the weight of the petroleum oil. Successful results may, however, be obtained with as little as .2% or as much as 2% or more of this or a similar

acting emulsifying agent, based on the weight of the oil.

The oils, emulsifying agent and water are thoroughly mixed in mixing tank 68, passed through pipe 16 to an emulsifying mill 17, and passed thence to a storage tank 18 from which the mixture proceeds through pipe 17 to the small compartment 63 of storage tank 41, valve 19 being provided to regulate the rate of flow.

The concentration of oleaginous material maintained in the coagulating liquid may vary considerably and is to a large extent determined by the results desired. Thus if it is desired that the oleaginous material not only inhibit depositions on the spinneret but also operate to remove insoluble impurities from the coagulating bath by sludge formation and to lubricate succeeding parts of the apparatus, such as guides, reels, etc., with which the thread comes into contact, a higher percentage of oleaginous material is desirable in the coagulating liquid than if the oleaginous material is required only to inhibit the formation of depositions on the spinnerets. A dispersion of from .3% to 3.0% of oleaginous material in the coagulating liquid will make possible the performance of all of the above-indicated functions. In practice, using the indicated oils, percentages between .5% and 1.5% have been found to provide the best results.

The coagulating liquid containing the finely dispersed oleaginous material is passed from small compartment 63 of storage tank 41 to coagulating trough 4: when, therefore, viscose is extruded through the spinnerets, the thread is formed in and coagulated by a coagulating liquid containing, besides the usual ingredients, a finely dispersed oleaginous material. As indicated above, the liquid leaving the coagulating trough returns to storage tank 41 by way of conduit 35, make-up tank 38, and conduit 39. Preferably, storage tank 41 is constructed so that large compartment 62 has a very large capacity, even several thousand gallons, so that the coagulating liquid is stored therein for a considerable period of time before it eventually overflows partition 64.

During this period of time the oil-laden impurities tend to form a sludge which usually floats on the top of the liquid in the large compartment 62 of storage tank 41 but which may, under certain conditions, settle to the bottom thereof, the intermediate portions of the liquid being ordinarily free from detrimental substances. Because of the arrangement of baffle plate 66, sludge floating on the surface of coagulating liquid in compartment 62 cannot flow over weir notch 65; consequently, only substantially uncontaminated liquid from beneath the surface, under the lower edge of baffle plate 66, flows on through the system. Baffle plate 66 thus serves to prevent the sludge from being recirculated with the rest of the coagulating liquid. Such sludge is removed continuously or from time to time, as desired; for example, the floating sludge which normally forms in large compartment 62 may be removed by scooping it from the surface of the liquid.

Under the conditions above described, the emulsion of oleaginous substance in the coagulating liquid is sufficiently stable to permit the emulsified liquid to pass from storage tank 41 to and through coagulating trough 4 and back to the large compartment 62 of storage tank 41 before the occurrence of any appreciable separation of the emulsion or the formation of an appreciable amount of sludge. Thus serious difficulties which

might otherwise be introduced by sludging of the impurities while the coagulating liquid is still in coagulating trough 4 are avoided. Indeed, the emulsion is so stable that it does not break even when a portion of the coagulating liquid passing to coagulating trough 4 is, as shown in Figure 3, diverted and passed through a coagulating liquid evaporator where it is subjected to an elevated temperature and a reduced pressure for a considerable time.

As an example, under the conditions above outlined, the coagulating liquid containing the emulsion formed as described may be subjected in evaporator 49 to evaporative conditions involving a vacuum of from 26 to 27 inches of mercury and a temperature of from 45 to 50° C. for an hour or more without breaking of the emulsion, during which period water in the amount of 15 to 20% of the original weight of liquid is removed.

At suitable intervals, storage tank 41 may be disconnected from the circulation system for cleaning, this being a simple matter if the circulating system includes several such storage tanks 41. To that end, valve 45 through which liquid passes from small compartment 63 of storage tank 41 is closed, as is valve 79 which supplies the emulsified oleaginous material to said compartment. Coagulating liquid flowing into storage tank 41 through conduit 39 is permitted to flow into small compartment 63 through weir notch 65. When the level of the liquid in compartment 63 reaches the lower edge of outlet duct 81, the lower edge of which outlet duct is below the top of partition 64, baffle plate 66 is removed and dam plate 82 substituted therefor.

As shown in Figure 5, dam plate 82 blocks weir notch 65, thus providing a substantially even surface along the top of partition 64. The liquid flowing from large compartment 62 into small compartment 63 then flows in a thin stream over the entire length of partition 64 carrying the floating sludge with it without creating undue turbulence, thus obviating dissemination of the sludge in the liquid in small compartment 63. All of the sludge passing into the small compartment 63 floats on the surface of the liquid therein and passes out through outlet duct 81; however, its removal may, if desired, be facilitated by scooping it out. When the liquid in storage tank 41 is substantially free of sludge, the valve 45 may be reopened, baffle plate 66 replaced, and valve 79 in pipe 67 reopened, after which the storage tank may be rejoined with the system.

Under the conditions above outlined, most of the agglomerated insoluble impurities such as sulfur which are present in the liquid contained in storage tank 41 find their way into the sludge which forms on the surface of the liquid in large compartment 62 of storage tank 41. A small amount of the petroleum oil separates from the emulsion in the form of a layer which floats on the surface of the coagulating liquid immediately beneath the sludge layer. When the sludge is scooped from the surface of the liquid in the tank or the tank is cleaned as above described, some of such separated oil may be removed.

It has been found that, under suitable circumstances, the colloidal impurities present in the coagulating bath, particularly colloidal sulfur, can be caused to aid the emulsifying agent in forming an emulsion so stable that substantially no oil separates even though the coagulating liquid requires several hours for circulation and is subjected to the aforementioned drastic con-

ditions in the evaporator. This can be accomplished by increasing the proportion of the oleaginous emulsifying agent to the other oleaginous substances employed. Thus, using the above-indicated substances, this result can be obtained by employing about 2% or more of the emulsifying agent based on the weight of the petroleum oil, which petroleum oil, as stated, is preferably in the neighborhood of 1% by weight of the coagulating liquid.

Under such a mode of operation, not only is the petroleum oil inhibited from separating from the emulsion, but the insoluble impurities such as sulfur, which apparently aid in maintaining the stability of the emulsion, precipitate from the emulsion only in storage tank 41. Since no petroleum oil is permitted to separate from the emulsion in the coagulating trough, very little, if any, is lost from the system other than that carried out of the coagulating bath by the thread; indeed, over a long period of time it is only necessary to add an emulsifying agent, and that rarely, to replace the amount carried out of the circulation system. In such case, storage tank 41 may be drained and cleaned from time to time in the manner indicated.

In the circumstances above described, the coagulating liquid therefore has finely dispersed therein, as by emulsification, a finely divided oleaginous material normally insoluble in the coagulating liquid. The thread is formed in the presence of such dispersed oleaginous material. The oleaginous material under conditions such as those described above inhibits, if not entirely prevents, the formation of harmful deposits of sulfur and/or other substances in and upon the spinnerets. In particular, it inhibits, if it does not entirely prevent, the formation of harmful crater-like deposits around the spinneret orifices. Which crater-like deposits arise primarily from insoluble impurities in the coagulating liquid, and the formation of harmful ring-like deposits in the spinneret orifices, apparently arising primarily from impurities in the viscose. Whatever deposits may form are soft, harmless, and easily removed.

Such oleaginous material also promotes the agglomeration of insoluble contaminants, such as sulfur, which are present in the coagulating liquid and facilitates their separation from the coagulating liquid either continuously or from time to time. The oleaginous material also lubricates the spinnerets and thread. In this connection, the oleaginous material carried by the thread forms films on the parts of the apparatus with which the thread comes into contact after leaving the spinneret, such as guides or reels, and inhibits the formation on such parts of the apparatus of precipitates or deposits of contaminants which would damage the thread by snagging or abrading it.

Under suitable circumstances, it is possible to obtain a desulfurizing action on the thread in the coagulating bath, so that considerable sulfur may be removed from the thread before it even leaves the coagulating bath.

Modifications may be made in the foregoing example of the preferred method of practicing the invention. The proportions of dispersing or emulsifying agent to the oleaginous material may be varied, depending upon the nature of the agent; indeed, two or more substances may act together to form the dispersing or emulsifying agent. Moreover, as indicated, the amount of oleaginous material dispersed in the coagulating

liquid is to a large extent dependent upon whether functions in addition to those of inhibiting spinneret depositions are desired of the oleaginous material. The example which follows is illustrative of another method of practicing the invention.

A soluble oil is made up consisting, by weight, of 50% refined petroleum oil of 30 seconds Saybolt viscosity at 100° F., 12% sorbitol monolaurate, and 38% of a 50% aqueous solution of modified ("solubilized") sorbitol monolaurate. The modified sorbitol monolaurate has been treated with ethylene oxide to render it soluble and is supplied by the Atlas Powder Company. A 10% aqueous dispersion is formed of this liquid, either by means of an emulsifying mill, as previously described, or merely by addition of the liquid to the desired quantity of warm water. The emulsion thus formed is added to the coagulating liquid. The unmodified sorbitol monolaurate and the modified sorbitol monolaurate cooperate efficiently to disperse the petroleum oil.

A very stable emulsion of the oleaginous material in the coagulating liquid is obtained which emulsion is, however, very effective even if only minute quantities of the oleaginous material are dispersed in the coagulating liquid. Fouling of spinnerets by the formation of deposits about or in the orifices is almost non-existent even though, by weight, less than 500 parts of the above-described soluble oil are dispersed in a million parts of coagulating liquid. Extremely good results in reduction of spinneret contamination have been obtained with dispersions of only 150 to 400 parts of said soluble oil in a million parts of coagulating liquid, only half of which soluble oil is mineral oil.

Because of the small amount of oleaginous material in the coagulating liquid under such circumstances, very little oleaginous material is carried out of the coagulating bath by the thread. In this case, it is desirable to remove insoluble impurities from the coagulating liquid by filtering or similar methods, since the amount of oleaginous material may be insufficient to permit the removal of such substances as a sludge. However, even such small quantities of oleaginous material cause some agglomeration of particles of impurities such as sulfur, thus facilitating the removal of such substances by filtering operations.

Similar results may be obtained with small quantities of the petroleum oils and the Sohio-X Soluble Oil used as the emulsifying agent in the first example. Likewise, the various functions other than that of inhibiting spinneret contamination described above in connection with the first example may be obtained by the use of a mixture of the type described in the second example provided that larger amounts of the mixture are employed. In such case, the amount of oil in the coagulating liquid is preferably within the range mentioned in connection with the first example.

In each of the two examples described above, moreover, it appears that more efficient action in inhibiting deposits in or about the spinneret orifices is obtained by the use of oils of lower viscosity numbers than by the use of oleaginous materials of higher viscosity numbers. Furthermore, it appears that the nature of the alloy of which the spinnerets are formed plays a part in the efficiency of the action of the dispersed oleaginous material in inhibiting depositions upon the spinnerets. Thus in each of the illustrated ex-

amples, spinnerets of 90% platinum and 10% rhodium are less likely to become contaminated than spinnerets formed of an alloy of 80% gold and 20% palladium. In either case, however, the number of spinnerets which must be replaced or cleaned as a result of contamination is far less when the present invention is employed than the number which must be cleaned or replaced in the absence of use of the present invention.

Various other modifications may be made in the methods and apparatus hereinabove described without departing from the spirit of the invention. The described oleaginous materials and emulsifying agents are not the only materials which may be employed for the purposes of the present invention. There may be employed one or more of several other organic or inorganic materials, preferably but not necessarily oleaginous, which are capable of being dispersed in the coagulating liquid and which, because of their nature, have an affinity for such insoluble impurities, even if of colloidal form, as are present in the coagulating bath.

Numerous types of substances, either soluble or insoluble in the coagulating liquid, may be employed as dispersing or emulsifying agents.

As examples of such agents may be mentioned the sulfated and sulfonated higher alcohols and esters, including the sodium or potassium salts of such sulfated and sulfonated hydrocarbons. Sulfated and sulfonated oils, either of the mineral, vegetable or animal types, may also be employed as dispersing or emulsifying agents. Examples are sulfonated petroleum, castor or coconut oils and the so-called Twitchell oils, each of which latter is made up of a base constituting a sodium salt of a sulfonated hydrocarbon dissolved in mineral oil. Some Twitchell oils are substantially insoluble in the coagulating liquid while others are soluble: both types make satisfactory emulsifying agents.

Certain esters of sulfodicarboxylic acids, such as the sodium salt of dilauryl sulfosuccinate sold as "Deceresol" by the American Cyanamid and Chemical Corporation, are also useful for dispersing agents in the practice of the invention. Sulfuric acid derivatives of certain amides, such, for example, as the compound having the formula



sold by the Colgate-Palmolive-Peet Corporation under the trade-mark "Arctic Syntex," are likewise efficient dispersing agents for the purposes of the present invention.

While the invention has been described in detail in connection with the manufacture of multiple filament viscose artificial silk thread by a continuous process, it is apparent that it is equally applicable to discontinuous processes, such as spool- and pot-spinning processes. Moreover, the invention is not restricted to the manufacture of viscose artificial silk thread. If desired, it may, at least in certain of its aspects, be applied to the manufacture of other products; e. g., strips, ribbons, tubes, sheets, etc., by processes which involve generally the extrusion of coagulable masses into liquid coagulants.

The term "spinneret," wherever employed in the claims, is intended to include other types of extrusion heads than the usual thread-forming spinnerets. The term "impurities" is intended to include such insoluble substances as sulfur, colloidal or otherwise, produced as a result of the coagulation reaction of the viscose thread.

It is also intended to include other insoluble substances in the coagulating liquid, together with substances such as silicates, hemi-celluloses or other substances which tend to form deposits on the spinnerets or in the orifices thereof.

It is intended that the patent shall cover, by suitable expression in the appended claims, whatever features of patentable novelty reside in the invention.

What is claimed is:

1. In the formation of cellulosic materials by the viscose process, the steps which comprise extruding viscose into an acidic coagulating liquid containing an emulsified petroleum oil which is substantially insoluble in said coagulating liquid, permitting said emulsified petroleum oil to form a sludge with impurities in the coagulating liquid and separating said sludge from the coagulating liquid.

2. In the formation of cellulosic materials by the viscose process, the steps which comprise extruding viscose into an acidic coagulating liquid containing an emulsifying agent and an emulsified petroleum oil which is substantially insoluble in said coagulating liquid, permitting said emulsified petroleum oil to form a sludge with impurities in the coagulating liquid and separating said sludge from the coagulating liquid.

3. In the formation of cellulosic materials by the viscose process, the steps which comprise extruding viscose into an acidic coagulating liquid containing a sulfonated hydrocarbon and an emulsified petroleum oil which is substantially insoluble in said coagulating liquid, permitting

said emulsified petroleum oil to form a sludge with impurities in the coagulating liquid and separating said sludge from the coagulating liquid.

5. The method of forming viscose thread which comprises extruding viscose into an acidic coagulating liquid containing an emulsified petroleum oil which is substantially insoluble in said coagulating liquid.

10 5. The method of forming viscose thread which comprises extruding viscose into an acidic coagulating liquid containing an emulsifying agent and an emulsified petroleum oil which is substantially insoluble in said coagulating liquid.

15 6. The method of forming viscose thread which comprises extruding viscose into an acidic coagulating liquid containing an emulsified petroleum oil which is substantially insoluble in said coagulating liquid and an emulsifying agent comprising a sulfonated hydrocarbon.

20 7. The method of forming thread by a wet-spinning process which comprises extruding a coagulable thread-forming mass into an acidic coagulating liquid containing an emulsified oleaginous substance which is substantially insoluble in said coagulating liquid and an emulsifying agent comprising a sulfonated hydrocarbon, permitting said oleaginous substance to form a sludge with impurities in the coagulating liquid

25 30 and separating said sludge from the coagulating liquid.

HAYDEN B. KLINE.

LOUIS S. FRYER.

ROBERT D. MACLAURIN.